

Dec. 11, 1945.

C. A. BRAUCHLER

2,390,867

PROCESS FOR FORGING CYLINDER HEADS

Filed March 31, 1943

7 Sheets-Sheet 1



Fig. 1



Fig. 2

Inventor

Charles A. Brauchler

By Grease and Bishop  
Attorneys

Dec. 11, 1945.

C. A. BRAUCHLER

2,390,867

PROCESS FOR FORGING CYLINDER HEADS

Filed March 31, 1943

7 Sheets-Sheet 2



Fig. 3



Fig. 6

Inventor

Charles A. Brauchler

By Grease and Bishop

Attorneys

Dec. 11, 1945.

C. A. BRAUCHLER

2,390,867

PROCESS FOR FORGING CYLINDER HEADS

Filed March 31, 1943

7 Sheets-Sheet 3



Inventor

Charles A. Brauchler

By Grease and Bishop

Attorneys

Dec. 11, 1945.

C. A. BRAUCHLER

2,390,867

PROCESS FOR FORGING CYLINDER HEADS

Filed March 31, 1943

7 Sheets-Sheet 4



Fig. 8



Fig. 7



21 Inventor

Charles A. Brauchler

By Grease and Bishop

Attorneys

Dec. 11, 1945.

C. A. BRAUCHLER

2,390,867

PROCESS FOR FORGING CYLINDER HEADS

Filed March 31, 1943

7 Sheets-Sheet 5



Fig. 9

Inventor

Charles A. Brauchler

By

Frease and Bishop

Attorneys

Dec. 11, 1945.

C. A. BRAUCHLER

2,390,867

PROCESS FOR FORGING CYLINDER HEADS

Filed March 31, 1943

7 Sheets-Sheet 6



Fig. 11



Fig. 12



Fig. 13

Inventor

Charles A. Brauchler

By Grease and Bishop

Attorneys

Dec. 11, 1945.

C. A. BRAUCHLER

2,390,867

PROCESS FOR FORGING CYLINDER HEADS

Filed March 31, 1943

7 Sheets-Sheet 7



Charles A. Brauchler  
By *Grease and Bishop*  
Attorneys

## UNITED STATES PATENT OFFICE

2,390,867

## PROCESS FOR FORGING CYLINDER HEADS

Charles A. Brauchler, Canton, Ohio

Application March 31, 1943, Serial No. 481,193

13 Claims. (Cl. 29—156.4)

The invention relates to the forging of cylinder heads and other parts from aluminum alloys and similar metals, and more particularly to a novel forging process in which the forgings are pressed rather than the usual practice of hammering.

The process is particularly concerned with the production of cylinder heads for aircraft engines, and to this end the present application illustrates and describes the invention as applied to the manufacture of cylinder heads for aircraft engines.

Under present practice these cylinder heads are cast from aluminum or aluminum alloys, such as duralumin, but the steady increase in the power output of aircraft engines, due to the present war effort, is rapidly approaching the point at which the cast heads will no longer be sufficiently strong to withstand greater pressures than those now generated within the cylinders.

The cooling fins on the conventional cast head have already reached a depth of about two and one-half inches, and any further increase in depth of these fins would greatly complicate the casting problem to a point where foundry rejects would be so high as to seriously retard production.

On the other hand, if a heavier casting were to be adopted, increased cooling area would necessarily have to be provided to dissipate the heat, and this in turn would necessitate a larger head requiring more space, and thus the vicious circle would continue, resulting in increasing the overall dimensions of the engine and adding to the weight of the airplane, thus reducing both its speed and load carrying capacity.

For this reason aircraft engineers, reluctant to increase the weight of the engines by making a more massive cylinder head, have been recently engaged in development work to produce a forging to replace the conventional cast cylinder head, because if a forging could be employed the increased tensile strength of the forged material over that of cast material would result in a cylinder head of twice the strength without any increase in weight or size while the greater thermal conductivity would considerably increase the cooling effect, and as the temperature of the cylinder head has a direct bearing on the power produced, this increased cooling of the head is of considerable importance.

A forged cylinder head would thus give planes a decided advantage in desert or tropical fighting and also permit the development of increased power at high altitudes. Further, the greater strength of the forging makes possible thinner walls around the intake and exhaust chambers,

permitting these chambers to be enlarged, resulting in increased power output and decreased fuel consumption, thus extending the range of operations of planes, so important in present day warfare.

However, a serious obstacle in the way of manufacturing these forged heads is the limited number of drop hammers in the country with sufficient power to produce these heads, and the heavy demands upon drop hammers for many other forged articles for war use. Since a minimum of nine hammer forging operations is required to produce one cylinder head forging and because it was found upon investigation that sufficient drop hammers to produce these forgings in any considerable numbers could not be obtained for about two years, it has been impossible up to the present time to equip airplane engines with forged cylinder heads.

Applicant however has overcome these obstacles and has developed the process embodied in the present invention, by which the forged cylinder heads are formed in a mechanical or hydraulic press in two operations, thus obtaining all of the advantages of the forged cylinder head without the use of drop hammers and with only a fraction of the labor and time required for drop forging the head; thereby freeing much needed drop hammers, as well as foundry equipment for other essential work.

It is therefore an object of the invention to provide a process for quickly and economically producing forgings for cylinder heads and the like by heating the metal to forging temperature and squeezing or pressing it in a mechanical or hydraulic press or the like, passing it in succession through two dies, the first die forming the rocker boxes and the second forming the outside contour of the head. The combustion recess may be formed by machining or may be formed in a third die, in an upsetting operation in which operation a skirt may be extruded around the combustion recess where desirable. The second and third steps may be combined in one operation by forming the outside contour of the head in suitable dies and simultaneously forming the combustion recess by means of a plunger while the forging is held in the forming dies.

Another object is to forge the cylinder head in the manner above mentioned from a blank or billet of bar stock extruded or rolled to the approximate or general shape of the head, or from a rectangular block or a cast ingot.

A further object of the invention is to provide a process for forging cylinder heads, and the like,

with a minimum of flash, thus preserving the original flow lines of the metal grain and producing a stronger finished product than that obtained by drop hammer forging where the flow lines curve outward towards the flash and are intersected during the machining operation.

The above objects and advantages, together with others which will be apparent from the drawings and following description, or which will be later referred to, may be attained by carrying out the improved forging process in the manner hereinafter described in detail and illustrated in the accompanying drawings, in which—

Fig. 1 is a perspective view of an extruded or rolled bar stock blank approximating the general shape of the cylinder head;

Fig. 2, a perspective view of the partly completed product after the first forging operation;

Fig. 3, a perspective view of the forged cylinder head after the second forging operation;

Fig. 4, an elevation partly in section of the forged cylinder head after the combustion recess has been formed therein and the skirt extruded as by a third operation upon an upsetting machine or the like;

Fig. 5, a bottom plan view of the forged cylinder head shown in Fig. 4;

Fig. 6, a perspective view of the finished forged head after the same has been machined;

Fig. 7, a vertical sectional view of the forging dies used in the first operation showing the dies in open position with a blank positioned therein ready for the first forging operation;

Figure 8 is a side elevation of the partly completed product produced in the dies shown in Fig. 7;

Figure 9 is a vertical sectional view of the dies for the second forging operation showing the same in open position with the partly completed forged product from the first operation positioned therein;

Fig. 10, a side elevation of the forged cylinder head as produced by the dies in the second operation;

Fig. 11, a vertical sectional view through a bar stock or ingot blank showing the grain flow of the metal;

Fig. 12, a vertical sectional view through the partly completed forged product of the first operation showing the grain flow;

Fig. 13, a similar view of the forged head as produced by the second operation, showing the grain flow; and

Fig. 14, a sectional view showing the dies and plunger for the upsetting operation.

Similar numerals refer to similar parts throughout the drawings.

In carrying out the improved forging process the cylinder head is forged from a blank of suitable size composed of an aluminum alloy which may be modified duralumin comprising substantially 90% aluminum and the balance made up of small amounts of several different metals.

This blank may be the usual substantially square block such as ordinarily used in hammer forging, or may be in the form of cast ingot, or if desired it may be extruded or rolled bar stock approximating the general shape of the head as indicated generally at 15 and as shown in detail in Figure 1, comprising the substantially rectangular body portion 16 and the oppositely disposed angular ribs 17 and 18 at two adjacent corners of the block for producing the rocker boxes at the inlet and exhaust sides of the cylinder head.

The first operation of the process is carried out in the lower and upper dies, shown at 19 and 20 respectively in Fig. 7, which are mounted in a heavy capacity hydraulic press, the lower die 19 being fixed upon the bed or table of the press and the upper die 20 being carried in the reciprocating ram of the press.

These dies are shaped as at 21 and 22 respectively, to form the rocker boxes upon the head, and the lower die may be provided with the bosses 23 for forming the intake and exhaust recesses in the head.

The blank, which may be of any of the shapes above referred to, is heated to forging temperature and placed in the lower die 19 as shown in Fig. 7 and the press is then operated to move the upper die 20 down upon the lower die. As the press may be of substantially 2500 tons capacity the heated blank will be squeezed under this extreme pressure to the contour of the dies producing the partially completed forged product indicated generally at 24 in Figs. 2, 8, 9 and 12.

In this first pressing operation the surface of the blank between the angular ribs 17 and 18 is partially rounded as indicated at 24a in Fig. 2, said ribs 17 and 18 being tapered toward each end and rounded at one end, the blank being recessed at the opposite end of the rib 17 as indicated at 24b and partially rounded at the corresponding end of the other rib as indicated at 24c so as to partially form rocker boxes 25 and 26 as indicated in Fig. 2, from the ribs 17 and 18 of the blank shown in Fig. 1 and this pressing operation may also include forming the enlarged oppositely tapered portion 27 upon one side of the partially completed product, just below the partially formed rocker box 26, this enlarged portion being for the purpose of cutting cooling fins in the cylinder head adjacent to the exhaust rocker box 26, and may also include the partial formation of inlet and exhaust ports 28 in the under side of the forging.

If the partially completed forged product still retains sufficient heat for further forging it may be immediately placed in the dies for the second operation shown in Fig. 9 and indicated respectively as the lower and upper dies 29 and 30, or if necessary the partially completed forging 24 may be reheated to forging temperature before it is placed in the dies for the second operation.

These dies are shaped as indicated at 31 and 31a respectively to produce the outside contour of the head when the press is operated to bring the dies together, squeezing the hot forging 24 to the finished shape indicated generally at 31 in Figs. 3, 10 and 13.

In this operation the top of the head is generally rounded as indicated at 32, the lower portion of the head is formed to generally circular shape as indicated at 33; the intake and exhaust recesses 28 are formed deeper into the head, and the same is recessed as at 34 adjacent to these recesses; the enlarged portion 27 at the exhaust side of the head is rounded; and the rocker boxes 25 and 26 are shortened and reduced to substantially the finished outside contour as indicated at 25a and 26a respectively, the ends thereof being further tapered and, if desired, bosses are formed thereon to form bearings for rocker shafts and the like.

The combustion recess 35 may be formed in the lower side of the head by machining, or if desired this operation may be more quickly accomplished in an upsetting operation, and in the event a skirt 36 is required at the bottom of

the head, as is customary in some type of engines, this skirt may be extruded in the same upsetting operation.

This upsetting operation may be carried out in apparatus such as shown in Fig. 14, which comprises generally a stationary lower die 44 mounted upon a bed 45, a vertically movable upper die 46 operated by a piston 47 of a hydraulic cylinder, or the like, and a plunger 48 operated by a piston 49 of a hydraulic cylinder, or the like.

The forging, as shown in Figs. 3 and 10, at forging temperature, is inserted through the opening 50 in the end plate 51, and placed in the lower die 44. The upper die 46 is then moved downward to the position shown in Fig. 14, holding the hot forging between the dies and the plunger 48 is moved inward, or toward the left as viewed in said figure forming the combustion recess 35 and extruding the skirt 36 around the same.

It has been found that, if desired, the production of these forgings may be further shortened by eliminating the step in which the forging shown in Figs. 3 and 10 is produced. For this purpose the partially completed product shown in Figs. 2 and 9, at forging temperature, may be placed in the lower die 44, shown in Fig. 14, and the upper die 46 is forced down, press forging the outer contour of the product to the shape shown in said figure.

The plunger 48 is then operated to form the combustion recess 35 in the forging and at the same time extrude the skirt 36, while the hot forging is held between the dies 44 and 46.

The finished forging as shown in Fig. 4, with the combustion recess and skirt formed thereon, may thus be produced in two, and a maximum of three operations, ready for machining to produce the finished cylinder head, as compared with a minimum of nine hammer forging operations to produce the same forging.

And it will be evident that the forging is completed without the use of drop hammers, of which there is an acute shortage during the present emergency, freeing the hammers for the production of other necessary products.

Cylinder heads forged by the improved process have a finer and more uniform grain structure in the metal than the conventional cast heads and have a more uniform grain flow pattern than hammer forged heads. This is due to the fact that excess metal is not squeezed out in a substantial flash as in drop hammer forging thus eliminating the outwardly curved flow lines which are intersected during the machining operation.

As shown in Figs. 11, 12 and 13 the flow line pattern of the head forged by this process is unbroken and substantially follows the outer contour of the forging, eliminating the usual outward curve toward the flash, which is intersected by machining resulting in weakening of the forged article.

As shown in Fig. 11 the grain flow, indicated at 31, is in a longitudinal direction and straight throughout the area of the blank. After the first forging operation, as shown in Fig. 12, it will be seen that the grain flow near the outside of the forging substantially follows the contour of the forging and is unbroken at the meeting surfaces of the dies where the relatively slight flash 38 is formed, this grain flow being indicated at 37a in Figure 12.

After the second forging operation, as shown in Fig. 13, the grain flow indicated at 37b is still

unbroken and follows the outside contour of the forging. This highly desirable flow grain pattern adds substantially to the strength of the finished cylinder head.

5 The finished forging may then be machined as shown in Fig. 6 cutting cooling fins, as indicated at 40, circumferentially around the lower portion 33 of the head and cutting cooling fins as indicated at 41 over the rounded upper portion 32 of the head between the rocker boxes 25a and 26a and cutting additional cooling fins 42 around the enlarged portion 27a on the exhaust side thereof.

15 The increased tensile strength over the cast head, without increase in weight or size, and the greater thermal conductivity of the forged metal substantially increases the cooling effect as much as 35%.

20 Furthermore, the increased strength of the forging achieved by the finer, more uniform and substantially unbroken grain structure in the metal makes possible thinner walls around the intake and exhaust chambers of the head, thus permitting these chambers to be enlarged producing an increase in power output and a decrease in fuel consumption, thus increasing the range, speed and load carrying capacity of planes equipped with these engines and at the same time substantially reducing the weight of the engine.

25 30 It has been found in actual practice that the horse power output of engines provided with these forged cylinder heads is increased as much as 15% while the weight is reduced as much as three and one-half pounds per cylinder, and in planes powered by four eighteen-cylinder motors it will be seen that this is a substantial reduction in weight.

35 40 Under present practice approximately 20% of the cast cylinder heads are rejected while it has been found that at least 95% of the forged heads pass the final inspection as finished parts of the airplane engines, thus substantially saving time, labor and material.

I claim:

45 1. The method of producing a forged engine cylinder head having thick walls for the formation of deep cooling fins, which consists in making the cylinder head solely by press forging and which comprises the steps of forming a substantially rectangular aluminum alloy blank having angular ribs at two adjacent corners thereof, heating said blank to forging temperature, forging the hot metal in one pressing operation said pressing operation including partially rounding the surface of the blank between said angular ribs, tapering the ribs toward each end, rounding one end of each rib, recessing the blank at the other end of one rib and partially rounding the blank at the corresponding end of the other rib so as to partially form said angular ribs into rocker boxes and then forging the hot, partially forged product exactly as produced by said first operation in a second pressing operation said second pressing operation including further rounding the upper portion of the head between the rocker boxes, substantially circularizing the lower portion of the head, shortening the rocker boxes and further tapering them at each end so as to form the entire finished outside contour of the head and the contour of the outer edges of the cooling fins entirely by forging.

60 65 70 75 2. The method of producing a forged engine cylinder head having thick walls for the formation of deep cooling fins, which consists in making the cylinder head solely by press forging and

which comprises the steps of forming a substantially rectangular aluminum alloy blank having angular ribs at two adjacent corners thereof, heating said blank to forging temperature, forging the hot metal in one pressing operation said pressing operation including partially rounding the surface of the blank between said angular ribs, tapering the ribs toward each end, rounding one end of each rib, recessing the blank at the other end of one rib and partially rounding the blank at the corresponding end of the other rib so as to partially form said angular ribs into rocker boxes and to partially form the outside contour of the head and then forging the hot, partially forged product exactly as produced by said first operation in a second pressing operation said second pressing operation including further rounding the upper portion of the head between the rocker boxes, substantially circularizing the lower portion of the head, shortening the rocker boxes and further tapering them at each end so as to form the entire finished outside contour of the head and the contour of the outer edges of the cooling fins entirely by forging.

3. The method of producing a forged engine cylinder head having thick walls for the formation of deep cooling fins, which consists in making the cylinder head solely by press forging and which comprises the steps of forming a substantially rectangular aluminum alloy blank having angular ribs at two opposite corners thereof, heating said blank to forging temperature, forging the hot metal in one pressing operation said pressing operation including partially rounding the surface of the blank between said angular ribs, tapering the ribs toward each end, rounding one end of each rib, recessing the blank at the other end of one rib and partially rounding the blank at the corresponding end of the other rib so as to partially form said angular ribs into rocker boxes and to partially form intake and exhaust recesses in the blank and then forging the hot, partially forged product exactly as produced by said first operation in a second pressing operation said second pressing operation including further rounding the upper portion of the head between the rocker boxes, substantially circularizing the lower portion of the head, shortening the rocker boxes and further tapering them at each end so as to form the entire finished outside contour of the head and the contour of the outer edges of the cooling fins entirely by forging and to deepen the intake and exhaust recesses.

4. The method of producing a forged engine cylinder head having thick walls for the formation of deep cooling fins, which consists in making the cylinder head solely by press forging and which comprises the steps of forming a substantially rectangular aluminum alloy blank having angular ribs at two opposite corners thereof, heating said blank to forging temperature, forging the hot metal in one pressing operation said pressing operation including partially rounding the surface of the blank between said angular ribs, tapering the ribs toward each end, rounding one end of each rib, recessing the blank at the other end of one rib and partially rounding the blank at the corresponding end of the other rib so as to partially form said angular ribs into rocker boxes and to partially form the outside contour of the head and to partially form intake and exhaust recesses in the blank and then forging the hot, partially forged product exactly

as produced by said first operation in a second pressing operation said second pressing operation including further rounding the upper portion of the head between the rocker boxes, substantially circularizing the lower portion of the head, shortening the rocker boxes and further tapering them at each end so as to form the entire finished outside contour of the head and the contour of the outer edges of the cooling fins entirely by forging and to deepen the intake and exhaust recesses.

5. The method of producing a forged engine cylinder head having thick walls for the formation of deep cooling fins which consists in making the cylinder head solely by press forging and which comprises the steps of heating an aluminum alloy blank to forging temperature, forging the hot metal in one pressing operation, said pressing operation including partially forming rocker boxes upon two adjacent corners of the blank, tapering said partially formed rocker boxes toward each end, rounding one end of each partially formed rocker box, recessing the blank at the other end of one partially formed rocker box and partially rounding the blank at the corresponding end of the other partially formed rocker box and rounding the surface of the blank between said partially formed rocker boxes, and then forging the hot, partially forged product exactly as produced by said first pressing operation in a second pressing operation, said second pressing operation including further rounding the upper portion of the head between the rocker boxes, substantially circularizing the lower portion of the head, shortening the rocker boxes and further tapering them at each end so as to form the entire finished outside contour of the cylinder head and rocker boxes thereon.

6. The method of producing a forged engine cylinder head having thick walls for the formation of deep cooling fins which consists in making the cylinder head solely by press forging and which comprises the steps of heating an aluminum alloy blank to forging temperature, forging the hot metal in one pressing operation, said pressing operation including partially forming rocker boxes upon two adjacent corners of the blank, tapering said partially formed rocker boxes toward each end, rounding one end of each partially formed rocker box, recessing the blank at the other end of one partially formed rocker box and partially rounding the blank at the corresponding end of the other partially formed rocker box, forming an enlarged, oppositely tapered portion upon one side of the blank just below one of the partially formed rocker boxes and rounding the surface of the blank between said partially formed rocker boxes, and then forging the hot, partially forged product exactly as produced by said first pressing operation in a second pressing operation, said second pressing operation including further rounding the upper portion of the head between the rocker boxes, substantially circularizing the lower portion of the head, shortening the rocker boxes and further tapering them at each end so as to form the entire finished outside contour of the cylinder head and rocker boxes thereon.

7. The method of producing a forged engine cylinder head having thick walls for the formation of deep cooling fins which consists in making the cylinder head solely by press forging and which comprises the steps of heating an aluminum alloy blank to forging temperature, forging the hot metal in one pressing operation, said

pressing operation including partially forming rocker boxes upon two adjacent corners of the blank, tapering said partially formed rocker boxes toward each end, rounding one end of each partially formed rocker box, recessing the blank at the other end of one partially formed rocker box and partially rounding the blank at the corresponding end of the other partially formed rocker box, partially forming inlet and exhaust ports in the under side of the blank, and rounding the surface of the blank between said partially formed rocker boxes, and then forging the hot, partially forged product exactly as produced by said first pressing operation in a second pressing operation, said second pressing operation including further rounding the upper portion of the head between the rocker boxes, substantially circularizing the lower portion of the head, deepening the inlet and exhaust ports, shortening the rocker boxes and further tapering them at each end so as to form the entire finished outside contour of the cylinder head and rocker boxes thereon.

8. The method of producing a forged engine cylinder head having thick walls for the formation of deep cooling fins which consists in making the cylinder head solely by press forging and which comprises the steps of heating an aluminum alloy blank to forging temperature, forging the hot metal in one pressing operation, said pressing operation including partially forming rocker boxes upon two adjacent corners of the blank, tapering said partially formed rocker boxes toward each end, rounding one end of each partially formed rocker box, recessing the blank at the other end of one partially formed rocker box and partially rounding the blank at the corresponding end of the other partially formed rocker box, forming an enlarged, oppositely tapered portion upon one side of the blank just below one of the partially formed rocker boxes and rounding the surface of the blank between said partially formed rocker boxes, and then forging the hot, partially forged product exactly as produced by said first pressing operation in a second pressing operation, said second pressing operation including further rounding the upper portion of the head between the rocker boxes, substantially circularizing the lower portion of the head, rounding the enlarged, oppositely tapered portion, shortening the rocker boxes and further tapering them at each end so as to form the entire finished outside contour of the cylinder head and rocker boxes thereon.

9. The method of producing a forged engine cylinder head having thick walls for the formation of deep cooling fins which consists in making the cylinder head solely by press forging and which comprises the steps of heating an aluminum alloy blank to forging temperature, forging the hot metal in one pressing operation, said pressing operation including partially forming rocker boxes upon two adjacent corners of the blank, tapering said partially formed rocker boxes toward each end, rounding one end of each partially formed rocker box, recessing the blank at the other end of one partially formed rocker box and partially rounding the blank at the corresponding end of the other partially formed rocker box, forming an enlarged, oppositely tapered portion upon one side of the blank just below one of the partially formed rocker boxes, partially forming inlet and exhaust ports in the under side of the blank, and rounding the sur-

face of the blank between said partially formed rocker boxes, and then forging the hot, partially forged product exactly as produced by said first pressing operation in a second pressing operation, said second pressing operation including further rounding the upper portion of the head between the rocker boxes, substantially circularizing the lower portion of the head, rounding the enlarged, oppositely tapered portion, deepening the inlet and exhaust ports, shortening the rocker boxes and further tapering them at each end so as to form the entire finished outside contour of the cylinder head and rocker boxes thereon.

15 10. The method of producing a forged engine cylinder head having thick walls for the formation of deep cooling fins which consists in making the cylinder head solely by press forging and which comprises the steps of heating an aluminum alloy blank to forging temperature, forging the hot metal in one pressing operation, said pressing operation including partially forming rocker boxes upon two adjacent corners of the blank, tapering said partially formed rocker boxes toward each end, rounding one end of each partially formed rocker box, recessing the blank at the other end of one partially formed rocker box and partially rounding the blank at the corresponding end of the other partially formed rocker box and rounding the surface of the blank between said partially formed rocker boxes, and then forging the hot, partially forged product exactly as produced by said first pressing operation in a second pressing operation, said second pressing operation including further rounding the upper portion of the head between the rocker boxes, substantially circularizing the lower portion of the head, shortening the rocker boxes and further tapering them at each end and, 20 forming bosses upon the rocker boxes so as to form the entire finished outside contour of the cylinder head and rocker boxes thereon.

11. The method of producing a forged engine cylinder head having thick walls for the formation of deep cooling fins which consists in making the cylinder head solely by press forging and which comprises the steps of heating an aluminum alloy blank having a longitudinal grain structure to forging temperature, forging the hot metal in one pressing operation, said pressing operation including partially forming longitudinally disposed rocker boxes upon two adjacent corners of the blank, tapering said partially formed rocker boxes toward each end, rounding 25 one end of each partially formed rocker box, recessing the blank at the other end of one partially formed rocker box and partially rounding the blank at the corresponding end of the other partially formed rocker box and rounding the surface of the blank between said partially formed rocker boxes, and then forging the hot, partially forged product exactly as produced by said first pressing operation in a second pressing operation, said second pressing operation including further rounding the upper portion of the head between the rocker boxes, substantially circularizing the lower portion of the head, shortening the rocker boxes and further tapering them at each end so as to form the entire finished outside contour of the cylinder head and rocker boxes thereon with substantially no flash whereby the flow line pattern of the grain of the metal is caused to conform to the contour of the head.

75 12. The method of producing a forged engine

cylinder head having thick walls for the formation of deep cooling fins which consists in making the cylinder head solely by press forging and which comprises the steps of heating an aluminum alloy blank having a longitudinal grain structure to forging temperature, forging the hot metal in one pressing operation, said pressing operation including partially forming longitudinally disposed rocker boxes upon two adjacent corners of the blank, tapering said partially formed rocker boxes toward each end, rounding one end of each partially formed rocker box, recessing the blank at the other end of one partially formed rocker box and partially rounding the blank at the corresponding end of the other partially formed rocker box and rounding the surface of the blank between said partially formed rocker boxes, and then forging the hot, partially forged product exactly as produced by said first pressing operation in a second pressing operation, said second pressing operation including further rounding the upper portion of the head between the rocker boxes, substantially circularizing the lower portion shortening the rocker boxes and further tapering them at each end so as to form the entire finished outside contour of the cylinder head and rocker boxes thereon and then forming a combustion chamber recess in the forged head by an upsetting operation with substantially no flash whereby the flow line pattern of the grain of the metal is caused to conform to the contour of the head.

13. The method of producing a forged engine cylinder head having thick walls for the forma-

tion of deep cooling fins which consists in making the cylinder head solely by press forging and which comprises the steps of heating an aluminum alloy blank having a longitudinal grain structure to forging temperature, forging the hot metal in one pressing operation, said pressing operation including partially forming longitudinally disposed rocker boxes upon two adjacent corners of the blank, tapering said partially formed rocker boxes toward each end, rounding one end of each partially formed rocker box, recessing the blank at the other end of one partially formed rocker box and partially rounding the blank at the corresponding end of the other partially formed rocker box and rounding the surface of the blank between said partially formed rocker boxes, and then forging the hot, partially forged product exactly as produced by said first pressing operation in a second pressing operation, said second pressing operation including further rounding the upper portion of the head between the rocker boxes, substantially circularizing the lower portion, shortening the rocker boxes and further tapering them at each end so as to form the entire finished outside contour of the cylinder head and rocker boxes thereon and then forming a combustion chamber recess in the forged head and simultaneously extruding a skirt around it by an upsetting operation with substantially no flash whereby the flow line pattern of the grain of the metal is caused to conform to the contour of the head.

CHARLES A. BRAUCHLER.